

June 14, 1960

G. P. TOUEY  
FIBROUS TOBACCO SMOKE FILTER CONTAINING  
FINELY DIVIDED SOLIDS  
Filed Feb. 8, 1956

2,940,456

FIG. 1.



FIG. 2.

FIG. 3



George P. Touey  
INVENTOR

BY  
Daniel I. Mayne  
John B. Hill, Jr.

ATTORNEYS

## 1

2,940,456

**FIBROUS TOBACCO SMOKE FILTER CONTAINING  
FINELY DIVIDED SOLIDS**

George P. Touey, Kingsport, Tenn., assignor to Eastman Kodak Company, Rochester, N.Y., a corporation of New Jersey

Filed Feb. 8, 1956, Ser. No. 564,172

10 Claims. (Cl. 131—208)

The present invention relates to tobacco smoke filtering material and elements thereof suitable for use in cigarettes, pipes, cigarette holders, and cigar holders. In connection with the consideration of the features described herein of spraying plasticizer in droplet form onto the continuous filaments and certain other details, reference may be made to Crawford and Stevens Patents 2,794,480 and 2,794,239.

In the aforementioned patents, newly discovered advantages of a certain type of fibrous tobacco smoke filter are discussed. The filter therein described is prepared from a specially conditioned tow of synthetically spun, crimped continuous filaments and comprises a structurally unitary, elongated rod-like mass of filaments and an annular wrapper encircling the mass, each filament of the mass being substantially coextensive therewith, the filaments being, in the aggregate, substantially parallel to each other and to the longitudinal axis of the mass with at least a large number of the individual filaments having a plurality of short portions thereof crimped into diverging and converging relationship to the main filament axis, a plurality of the filaments having surface solvation bonds to contiguous filaments at random points of contact. Very good results have been obtained in the use of such filters for the removal of nicotine and tars from tobacco smoke, especially in view of the fact that the filters supply other requirements, such as a unitary nature, rigidity, and resiliency, which are equally as necessary to the success of a tobacco smoke filter.

These filters also have a marked processing advantage over other filters known in the art. However, since the filaments in such filters are generally parallel to each other, some channeling of the smoke through the filter may be possible.

In other words, while a desirable amount of interference with the smooth flow of combustion products through the channels is provided by the random bonds between adjacent filaments, by the incompleteness of filament orientation, and by the short filament portions which are crimped into diverging and converging relationship to the main filament axis, yet a limited amount of the smoke passing through the filter apparently travels through channels in a smooth, non-turbulent and undisturbed manner and thereby may be exposed to somewhat less than a theoretically maximum amount of impingement upon and contact with the solid surfaces of the filter. Experimental investigations have shown that any attempt to reduce the size or change the shape of the detrimentally smooth smoke channels through the filters by an increase in filter density either through greater compaction of the filament mass or through the use of finer filaments generally also results in an intolerable increase in pressure drop through the filter. It is also unsatisfactory to substantially increase the amount of filament crimp in order to obtain an increase in the amount of smoke impinge-

## 2

ment by increasing the number of divergent and convergent filament portions. Additional crimp may weaken the filaments to the extent that they will not be able to withstand the tension which is applied to obtain tow bonding according to the Crawford and Stevens method.

In my copending U.S. patent application Ser. No. 413,950 filed March 3, 1954, now Patent No. 2,881,769, of which the present application is a continuation in part, I have disclosed and claimed an improvement based on

10 my discovery that the efficiency of filters of the type described above may be substantially increased without the expected equivalent increase in pressure drop through the filters by preparing the filters with deposits of finely divided solid vegetable starch particles in the smoke channels provided by the spacing of adjacent filaments. The starch particles are carried by and supported on the surfaces of the filaments or fibers.

I have now discovered that a novel additive comprising one of certain inorganic salts provides a filtration efficiency equally as high as the starches and exhibits an advantageous distinction in that it is capable of neutralizing gaseous acids, e.g. acetic acid, contained in the smoke and of serving as a buffering material for maintaining the pH of the smoke in the desired range, i.e. within 25 the range of 6.5 to 7.5. I have further found that these salts may be applied as finely divided solids from a slurry in a substantially non-volatile liquid plasticizer for the filament material.

This invention, therefore, has as one object the production 30 of an efficient cigarette smoke filter consisting of a filamentary filtering material, particularly a material comprising an elongated, cylindrical bundle of substantially parallel and longitudinally aligned textile fibers infused with finely divided particles of certain inorganic salts.

35 Another object is to provide means for increasing the efficiency of a cigarette filter prepared from a textile fiber. A still further object is provision of a filter which is capable of removing nicotine, tars, and other deleterious components of cigarette smoke without causing the smoke

40 to be dry or distasteful. Another object is to increase the efficiency of tobacco smoke filters of the Crawford and Stevens patents without creating a high pressure drop. A further object is to provide a filter which not only removes particulate liquids and solids from the smoke but

45 also buffers the pH of the smoke. Still another object is to provide a firmly adhering particulate additive for fibrous tobacco smoke filters, particularly those filamentary filters prepared with filaments bonded through a coalescence obtained by means of the application of a

50 spray of a liquid, solvent-type plasticizer. A further object is to provide a method of applying a powdered additive to a fibrous filter through the medium of a spray of a slurry of the additive in a liquid plasticizer. Other objects will be obvious from the present specification and

55 claims.

In accordance with the present invention, the fibers of a pervious fibrous filter mass are made to carry a dispersed deposit of a finely divided, solid, inorganic salt selected from the group consisting of the phosphates and 60 carbonates of magnesium and calcium. Accordingly, the present invention consists, in general, in a fibrous tobacco smoke filtering medium comprising a mass of fibers, the spacing of the fibers providing minute passages for smoke through the mass, the mass carrying therein an additive comprising finely divided solid particles of a water-in-

65 soluble inorganic salt of the type described above in an amount of about 5% to about 60% by weight of the fibers plus additive (the concentration not being critical so long as there is sufficient additive present to improve the 70 filtration efficiency of the filter without creating excessive

pressure drop), said particles being supported along the surfaces of and by the fibers and occupying positions along the walls of and partially blocking said passages whereby a substantial portion of the smoke is impinged on the particles.

A more specific and very advantageous embodiment of the invention comprises a new tobacco smoke filtering material of synthetically spun continuous crimped thermoplastic filaments and an element made therefrom, the element comprising a structurally unitary elongated, cylindrical rod-like mass of filaments and an annular wrapper encircling the mass, each filament of the mass being substantially coextensive therewith, the filaments in the aggregate being in substantial parallel disposition with each other and with the longitudinal axis of the mass but at least a plurality of the filaments each having a plurality of short portions crimped into diverging and converging relationship to the main filament axis, a plurality of the filaments having surface solvation bonds to contiguous filaments at random points of contact, the mass carrying uniformly dispersed therein an additive in the amount of about 5% to about 60% by weight of the mass plus additive, the additive being a water-insoluble inorganic salt selected from the group consisting of magnesium and calcium salts of ortho-, meta- and pyro-phosphoric acids and carbonic acid.

Most advantageously, the invention comprises a filter of cellulose acetate fibers having surface solvation bonds achieved through the application of a plasticizer spray, the filter carrying uniformly dispersed water-insoluble inorganic salt particles in the amount of about 5 to 30% by weight of the filter.

Any suitable means known to the art for spreading a powder onto a fibrous surface or through a fibrous mass may be employed in preparing filters of the invention. Thus, for example, the inorganic salt powder can be blown onto the fibers or it can be applied as a slurry in cold water or in a volatile organic vehicle. Another method is to apply the powder to the fibers electrostatically, i.e. to induce a charge on the fibers by friction or other suitable means and then to run the fibers through a chamber containing a highly concentrated cloud of salt dust. Preferably this is done with the fibers or filaments in the form of a tow and in a banded, i.e. spread-out condition. Still another method for applying the salt particles is to wet the surface of the filaments with an adhesive or a plasticizer before exposing them to a solids dusting device or other solids applicator. The powder then may be continuously applied to an opened and banded moving tow formed as described in the Crawford and Stevens patents. That is to say, tow from a supply roll is opened to debundleize the filaments and provide a larger and more uniform tow cross section, and the opened tow is spread uniformly to a much larger width of e.g., 10 times its original width, thereby exposing substantially all of the filaments to material, i.e. plasticizer, issuing from a dispenser adjacent which the tow passes. The dust may be added before, simultaneously with, or after the plasticizer, preferably with or after, and most advantageously with the plasticizer. In the latter case the plasticizer first is converted to a slurry containing the finely divided inorganic salt and, if necessary, a diluent such as water or alcohol. The diluent must be a non-solvent for the powder but may dissolve, in or emulsify with the plasticizer. I have found that finely divided solids which have a tendency to sift out of fibrous filter masses generally are more firmly bound if applied in a plasticizer slurry. Also, by use of a slurry for application of the solid it has been possible to load the fibers with larger concentrations of uniformly dispersed and firmly bound additive. Employment of a diluent inert to the powder and to the fiber is valuable in facilitating application of larger quantities of additive without a corresponding increase in the quantity of plasticizer.

The invention is illustrated in the accompanying drawings in which:

Fig. 1 represents a magnified view of the interior of a mass of filtering material prepared in accordance with the invention,

Fig. 2 is a view of a cigarette having attached thereto a tip prepared from a filtering material of the invention, and

Fig. 3 represents a considerably magnified view of a section of filaments, such as a section of filaments from Fig. 1. Fig. 3 illustrates how a suspension of plasticizer with powdered additive (as will be described hereinafter) when sprayed on the crimped continuous filaments as droplets, causes the deposit of the additive on the surface of the filaments.

In further detail and referring to Fig. 3, the crimped continuous filaments are shown at 5, 6 and 7, for example. The powdered additive of the present invention is illustrated at 8, 9 and 10, for example. The powdered additive will be carried by the crimped continuous filaments where the aforementioned suspension of plasticizer and additive droplets come in contact with the filaments. The plasticizer being compatible with the filaments may migrate into the surface of the filaments or otherwise soften spots on the surface of the filaments so that the powdered additive of the present invention is affixed to the surface of the filaments at that point. Also, where plasticizer droplets contact adjacent filaments and crossing filaments, as illustrated at 11, 12 and 13, because of the softening action of the plasticizer the filaments will bond to one another at random points.

The invention is further illustrated in the following examples:

#### EXAMPLE 1.—MAGNESIUM CARBONATE

A partially opened tow of a crimped, regular cross-section cellulose acetate yarn (39.2% acetyl) having about eight crimps per inch and containing approximately 10,000 filaments of 8 denier per filament was slowly pulled over a compressed air banding device as disclosed in the aforementioned Crawford and Stevens patents and in Jackson, U.S. Patent 2,737,688, which spread out the filaments to a width of about twelve inches. While the tow was in this spread condition it was sprayed (using a conventional point spray gun) uniformly with finely divided droplets of di(methoxyethyl) phthalate plasticizer in order to make numerous portions of the surfaces of the filaments soft and tacky. The spread tow was then passed through a dusting chamber which dusted the fibers uniformly with a finely divided (325 mesh) powder of magnesium carbonate ( $MgCO_3$ ) of a type commercially available from Baker Chemical Co. and designated as analytical grade. On leaving the dusting chamber the tow contained 14% plasticizer and 18% magnesium carbonate, based on the total weight of tow, carbonate and plasticizer. After this spreading, spraying, and dusting, the treated tow was pulled back to its original shape of a compact bundle, i.e. cord, and fed into a conventional cigarette filter plug making machine which formed it cylindrically, wrapped it with paper, and cut it into rods 78 mm. in length and 7.5 mm. in diameter. The rods were then given a heat treatment for one hour at 80° C. to cause partial solvation of the acetate filaments by the plasticizer and thereby bond the carbonate particles to the filaments and the filaments to each other, imparting firmness to the rods. Thereupon the rods were readily cut into 13 mm. filter tip lengths and attached to king-size (85 mm.) cigarettes of a standard brand available on the retail market in the U.S. The cigarettes were first shortened by 13 mm. and the 13 mm. rods then affixed to the shortened cigarettes by means of an adhesive tape. These filter cigarettes were smoked to a total butt length of 35 mm. on a smoking machine similar in design and operation to the smoking

machine described by J. A. Bradford, W. R. Harlan and H. R. Hanmer in Industrial and Engineering Chemistry, vol. 28, pp. 836-9 (1936). The smoke which passed through the cigarettes was collected and analyzed for nicotine and tar content.

Control filters without a powdered additive were also prepared from the same cellulose acetate tow containing the same amount of di(methoxyethyl) phthalate plasticizer. These filters were attached to the same brand of standard king size cigarettes shortened by 13 mm. These cigarettes were also smoked to a total butt length of 35 mm. by means of the smoking machine. The smoke which passed through the cigarettes was collected and analyzed for nicotine and tar content.

Ten unfiltered king size cigarettes (same brand) which were not shortened by 13 mm. were smoked to a butt length of 35 mm. by means of the smoking machine. The smoke which passed through the cigarettes was collected and analyzed for nicotine and tar content.

The results obtained from the three sets of cigarettes 20 are listed in Table I.

Table I

|                                                               | Average Pressure Drop, inches | mg. Tars Found in the Smoke | mg. Nicotine Found in the Smoke |
|---------------------------------------------------------------|-------------------------------|-----------------------------|---------------------------------|
| Cigarettes without filters (85 mm. length)                    | 3.5                           | 163                         | 25                              |
| Cigarettes with cellulose acetate filters                     | 4.0                           | 148                         | 23                              |
| Cigarettes with cellulose acetate-magnesium carbonate filters | 4.2                           | 92                          | 14                              |

Pressure drop is expressed above in inches of water at an air flow rate of 17.5 cc./sec. through the cigarette.

From the results listed above it can be seen that the filter containing the combination of acetate fibers and magnesium carbonate reduced the amount of tar collected by 43.6% and the amount of nicotine collected by 44%. The control filter reduced the amount of tars collected by 9.2% and the amount of nicotine collected by 8%. The increase in pressure drop of the filtered cigarette due to the addition of the carbonate to the filter was only about 5%.

#### EXAMPLE 2.—CALCIUM CARBONATE

The procedures described in Example 1 were repeated using the same tow of cellulose acetate and the same plasticizer but using in place of the magnesium carbonate a powdered calcium carbonate ( $\text{CaCO}_3$ ) capable of passing through a 325-mesh screen. The treated tow contained 14% plasticizer and 20% calcium carbonate (based on the total weight of the treated tow) as it left the dusting chamber. The baked plugs were cut into 13 mm. filter tips and attached to the standard king size cigarettes which had been shortened by 13 mm. These filtered cigarettes were smoked to a total butt length of 35 mm. on the smoking machine operated under the same conditions as in Example 1, and the smoke which passed through the cigarettes was collected and analyzed for nicotine and tar content.

The collected smoke contained 90 milligrams of tar and 13 milligrams of nicotine. This corresponds to a reduction in tar of 44.6% and a reduction in nicotine of 48.0% due to the filter. The cigarettes had an average pressure drop of 4.3 inches of water.

#### EXAMPLE 3.—CALCIUM CARBONATE

The procedures described in Example 1 were repeated using a tow of cellulose acetate yarn containing 5,000 75

filaments of 16 denier per filament, a plasticizer consisting of triethyl citrate, and a powder consisting of calcium carbonate ( $\text{CaCO}_3$ ) with an average particle size of 0.1 micron (Multifex MM, Diamond Alkali Company).

5 The treated tow contained 60% cellulose acetate, 30% calcium carbonate, and 10% plasticizer. A control tow of cellulose acetate yarn of 5,000 filaments, 16 denier per filament, and containing 14% triethyl citrate, was also prepared. Both treated tow samples were processed into filter rods and the rods were heated at 60° C. for 1 hour. Filter tips of 13 mm. in length were prepared from both sets of rods and placed on the standard king size cigarettes which had been shortened by 13 mm. Ten cigarettes containing the calcium carbonate filters and 10 cigarettes containing the control filters were smoked to butt lengths of 35 mm. on the smoking machine. The smoke which passed through the cigarettes was collected and analyzed for nicotine and tar content.

|                                                                    | Average Pressure Drop, inches | mg. Tars Found in the Smoke | mg. Nicotine Found in the Smoke |
|--------------------------------------------------------------------|-------------------------------|-----------------------------|---------------------------------|
| Cigarettes with cellulose acetate filter (85 mm. length)           | 3.8                           | 155                         | 24                              |
| Cigarettes with cellulose acetate- $\text{CaCO}_3$ (85 mm. length) | 4.1                           | 115                         | 18                              |

30 From the values listed above and in Example 1 it can be seen that the filter containing the combination of acetate fibers and calcium carbonate reduced the amount of tars collected by 29.4% and the amount of nicotine collected by 28.0%. The control filter reduced the amount of tars collected by 4.9% and the amount of nicotine collected by 4.0%. The increase in pressure drop of the filtered cigarette due to the addition of the calcium carbonate to the filter was only about 5%.

#### EXAMPLE 4.—CALCIUM CARBONATE

A tow of regenerated cellulose yarn (viscose) containing 16,000 filaments of 6 denier per filament was spread out to a width of 10 inches and sprayed with a 25% aqueous solution of dextrin glue. While the tow was still spread out and wet with the glue it was passed through a dusting chamber where it was uniformly covered with a fine calcium carbonate dust of 0.1 micron particle size (Multifex MM). On leaving the dusting chamber the tow consisted of 40 parts regenerated cellulose fibers, 30 parts glue (25% solution) and 30 parts calcium carbonate. The combination was pulled back into the form of a compact bundle or cord and fed into a filter-rod making machine which paper wrapped it and cut it into filter plugs 78 mm. in length and 7.5 mm. in diameter. The rods were heated for 1 hour at 100° C. to dry the glue and bond the powder to the fibers. 50 The plugs were then cut into 13-mm. filter tip lengths and attached to 85 mm. standard king size cigarettes which had been shortened by 13 mm. Ten of these cigarettes were smoked to a total butt length of 35 mm. on the smoking machine. The smoke which passed through 55 the cigarettes was collected and analyzed for nicotine and tar content.

A control tow sample, consisting of 16,000 filaments of the 6 denier per filament regenerated cellulose and containing 43% of dextrin glue (25% solution) but no 60 calcium carbonate, was prepared in a similar manner. The plugs from this tow were heated for 1 hour at 100° C. and cut into filter tips 13 mm. in length. These tips were attached to 85 mm. standard king size cigarettes which had been shortened by 13 mm. Ten of these cigarettes were smoked to a total butt length of 75

35 mm. on the smoking machine. The smoke which passed through the cigarettes was collected and analyzed for nicotine and tar content.

|                                                                                    | Average Pressure Drop, inches | mg. Tars Found in the Smoke | mg. Nicotine Found in the Smoke |
|------------------------------------------------------------------------------------|-------------------------------|-----------------------------|---------------------------------|
| Cigarettes with the regenerated filter (85 mm. length)                             | 4.1                           | 140                         | .21                             |
| Cigarettes with the regenerated cellulose-CaCO <sub>3</sub> filter (85 mm. length) | 4.3                           | 100                         | .16                             |

From the values listed above and in Example 1 it can be seen that the filter containing the combination of regenerated cellulose fibers and calcium carbonate reduced the amount of tars collected by 38.7% and the amount of nicotine collected by 36.0%. The control filter of regenerated cellulose fibers reduced the amount of tars collected by 14.1% and the amount of nicotine collected by 16.0%. The increase in the pressure drop of the filtered cigarette due to the addition of the calcium carbonate to the filter was only about 5%.

#### EXAMPLE 5.—CALCIUM CARBONATE

A tow of cellulose acetate yarn containing 12,000 filaments of 5 denier per filament was spread to a width of 12 inches and sprayed with an emulsion consisting (by weight) of 0.03 part sodium lauryl sulfate, 1 part di(methoxyethyl)phthalate plasticizer, 2 parts water, and 3 parts calcium carbonate powder of ultimate particle size of approximately 6 microns. The spread tow was then pulled back into a compact bundle or cord and fed into a cigarette filter plug making machine which paper wrapped it and cut it into filter rods 78 mm. in length and 8 mm. in diameter. The rods were heated for thirty minutes at 100° C. to evaporate the water and to bond the calcium carbonate firmly to the fibers by means of the plasticizer. Analyses of the plugs indicated that they consisted of 51% cellulose acetate fibers, 33% calcium carbonate, 5% moisture, and 11% di(methoxyethyl)phthalate plasticizer. The heated and cooled plugs were quite firm and the calcium carbonate was firmly bonded to the fibers. The plugs were cut into 13-mm. filter tip lengths and attached to standard American king size (85 mm.) cigarettes which had been shortened by 13 mm. These filtered cigarettes were smoked to a total butt length of 35 mm. on the standard smoking machine described in Example 1. The smoke which passed through the cigarettes was collected and analyzed for nicotine and tar content.

A tow of cellulose acetate yarn containing 20,000 filaments of 5 denier per filament was spread to a width of 12 inches and sprayed with an emulsion consisting of 0.03 part sodium lauryl sulfate, 1 part di(methoxyethyl)phthalate plasticizer, and 2 parts water. This tow, containing no calcium carbonate, was converted into filter plugs in the manner described above and the plugs were dried for thirty minutes at 100° C. Analyses of these plugs indicated that they consisted of 84% cellulose acetate fibers, 12% di(methoxyethyl)phthalate plasticizer, and 4% moisture. The plugs were cut into 13-mm. filter tips and attached to ten standard king size cigarettes shortened by 13 mm. These cigarettes were also smoked to total butt lengths of 35 mm. on the smoking machine. The smoke which passed through the cigarettes was collected and analyzed for nicotine and tar content.

Ten unfiltered, standard king size cigarettes which were not shortened by 13 mm. were smoked to a butt length of 35 mm. by means of the smoking machine. The smoke which passed through the cigarettes was collected and analyzed for nicotine and tar content.

The results obtained from the three sets of cigarettes are listed in Table II.

|                                                                                     | Average Pressure Drop, <sup>1</sup> inches | mg. Tars Found in the Smoke | mg. Nicotine Found in the Smoke |
|-------------------------------------------------------------------------------------|--------------------------------------------|-----------------------------|---------------------------------|
| Unfiltered cigarettes (85 mm.)                                                      | 3.3                                        | 165                         | 25                              |
| Cigarettes, 72 mm. in length, containing 13-mm. acetate filter of 20,000 filaments. | 4.2                                        | 130                         | 20                              |
| Cigarettes, 72 mm. in length, containing 13-mm. acetate-CaCO <sub>3</sub> filter    | 4.2                                        | 93                          | 13                              |

<sup>1</sup> Pressure drop in inches of water at an air flow rate of 17.5 cc./second through the cigarette.

From the results listed above, it can be seen that the filter containing the combination of cellulose acetate fibers and calcium carbonate reduced the amount of tars collected by 44% and the amount of nicotine collected by 48%. The filter containing the larger number of cellulose acetate fibers but no calcium carbonate reduced the amount of tars by only 21% and the amount of nicotine by 20%, although its average pressure drop was equal to that of the cellulose acetate-calcium carbonate filter.

#### EXAMPLE 6.—CALCIUM CARBONATE

A tow of cellulose acetate yarn containing 14,000 filaments of 5 denier per filament was spread to a width of 12 inches and sprayed with a suspension of 51% calcium carbonate powder in di(methoxyethyl)-phthalate plasticizer containing 33% ethyl alcohol. The calcium carbonate powder had an ultimate particle size of 3 microns.

The spread tow was pulled back into a compact bundle or cord and fed into a cigarette filter plug making machine which paper wrapped it and cut it into filter rods 78 mm. in length and 8 mm. in diameter. The rods were heated for thirty minutes at 80° C. to evaporate the ethyl alcohol and bond the calcium carbonate powder to the fibers by means of the plasticizer. Analyses of the plugs indicated that they consisted of 65% cellulose acetate fibers, 20% calcium carbonate powder, and 13% plasticizer. The heated and cooled plugs were quite firm and the calcium carbonate was firmly bonded to the fibers. The plugs were cut into 13-mm. filter tips and attached to standard American king size cigarettes which had been shortened by 13 mm. These filtered cigarettes were smoked to a total butt length of 35 mm. on the standard smoking machine described in Example 1. The smoke which passed through the cigarettes was collected and analyzed for nicotine and tar content.

The collected smoke contained 111 mg. of tar and 15 mg. of nicotine. This corresponds to a reduction in tar of 33% and a reduction in nicotine of 40% due to the filter when the values obtained are compared with the unfiltered cigarette values listed in Example 5. The filtered cigarettes had an average pressure drop of 4.3 inches of water.

#### EXAMPLE 7.—CALCIUM CARBONATE

A tow of cellulose acetate yarn containing 14,000 filaments of 5 denier per filament was spread to a width of 12 inches and sprayed with a suspension of 58% calcium carbonate powder in glycerol tripropionate plasticizer. The calcium carbonate powder had an ultimate particle size between 7 and 10 microns.

The spread tow was pulled back into a compact bundle or cord and fed into a cigarette filter plug making machine which paper wrapped it and cut it into filter rods 78 mm. in length and 8 mm. in diameter. Within one hour at room temperature the rods were rigid and the calcium carbonate was firmly bonded to the fibers. The plugs were cut into 13 mm. filter tips and attached to standard king size cigarettes which had been shortened by 13 mm. These filtered cigarettes were smoked

to a total butt length of 35 mm. on the standard smoking machine described in Example 1. The smoke which passed through the cigarettes was collected and analyzed for nicotine and tar content.

The collected smoke contained 108 mg. of tar and 15 mg. of nicotine. This corresponds to a reduction in tar of 35% and a reduction in nicotine of 40% due to the filter when the values are compared with the unfiltered cigarette values listed in Example 5. The filtered cigarettes had an average pressure drop of 4.2 inches of 10 water.

**EXAMPLE 8.—MAGNESIUM PHOSPHATE**  
[ $Mg_3(PO_4)_2$ ]

A tow of the type employed in Example 1 was treated 18 as described in that example with magnesium phosphate (325 mesh) rather than magnesium carbonate as employed in Example 1. On leaving the dusting chamber, the tow of fibers contained 14% plasticizer and 18% magnesium phosphate based on the total weight 20 of the combination. Filters were made from this treated tow and fastened to cigarettes which were then test smoked, all by methods as described in Example 1. Analytical data obtained showed that cigarettes with cellulose acetate-magnesium phosphate filters (85 mm. length) had an average pressure drop of 4.2 inches. The smoke contained 98 mg. of tars and 15 mg. nicotine. Comparison of this data with the data obtained for 25 control filters and unfiltered cigarettes in Example 1 shows that the magnesium phosphate filter reduced the amount of tars collected by 40.0% and the amount of nicotine by 40.0%. The increase in pressure drop of the filtered cigarettes due to the addition of the magnesium phosphate to the fiber was only about 5%.

**EXAMPLE 9.—CALCIUM PHOSPHATE**  
[ $Ca_3(PO_4)_2$ ]

The procedures described in Example 1 were repeated using the same tow of cellulose acetate and the same plasticizer but using a powdered calcium phosphate  $Ca_3(PO_4)_2$  capable of passing through a 325-mesh screen in the dusting chamber. The tow of fibers prepared in this case contained 14% plasticizer and 20% calcium phosphate (based on the total weight) as it left the dusting chamber. The baked plugs were cut into 13-mm. filter tips and attached to the standard king size cigarettes which had been shortened by 13 mm. These filtered cigarettes were smoked to a total butt length of 35 mm. on the smoking machine and the smoke which passed through the cigarettes was collected and analysed for nicotine and tar content.

The collected smoke contained 100 milligrams of tar and 16 milligrams of nicotine. This corresponds to a reduction in tar of 38.6% and a reduction in nicotine of 36.1% due to the filter. The cigarettes had an average pressure drop of 4.4 inches of water.

**EXAMPLE 10.—CALCIUM PYROPHOSPHATE**  
[ $Ca_2P_2O_7$ ]

The procedures described in Example 1 were repeated using a tow of cellulose acetate yarn containing 5,000 filaments of 16 denier per filament, a plasticizer consisting of triethyl citrate, and a powder consisting of calcium pyrophosphate,  $Ca_2P_2O_7$ , capable of passing through a 325-mesh screen. The treated tow contained 60% cellulose acetate, 30% calcium salt, and 10% plasticizer. A control tow of cellulose acetate yarn of 5,000 filaments, 16 denier per filament, and containing 14% triethyl citrate, was also prepared. Both treated tow samples were processed into filter rods and the rods were heated at 60° C. for one hour. Filter tips of 13 mm. in length were prepared from both sets of rods and placed on the standard king size cigarettes which had been shortened by 13 mm. Ten cigarettes containing the calcium pyrophosphate filters and 10 cigarettes containing the control filters were 70

smoked to butt lengths of 35 mm. on the smoking machine. The smoke which passed through the cigarettes was collected and analyzed for nicotine and tar content. Results were as shown in Table III.

*Table III*

|                                                                           | Average Pressure Drop, inches | mg. Tars Found in the Smoke | mg. Nicotine Found in the Smoke |
|---------------------------------------------------------------------------|-------------------------------|-----------------------------|---------------------------------|
| Cigarettes with cellulose acetate filter (85 mm. length)                  | 3.8                           | 155                         | 24                              |
| Cigarettes with cellulose acetate-<br>$Ca_2P_2O_7$ filter (85 mm. length) | 4.2                           | 110                         | 17                              |

From the values listed above and in Example 1, it can be seen that the filter containing the combination of acetate fibers and calcium pyrophosphate reduced the amount of tars collected by 32.6% and the amount of nicotine collected by 32.0%. The control filters reduced the amount of tars collected by 4.9% and the amount of nicotine collected by 4.0%. The increase in pressure drop of the filtered cigarette due to the addition of the calcium pyrophosphate to the filter was only about 5%.

**EXAMPLE 11.—CALCIUM DIPHOSPHATE**  
[ $CaHPO_4$ ]

A tow as described in Example 4 was treated and converted into filters as described in that example, except that calcium diphosphate (capable of passing through a 325 mesh screen) was used in place of the calcium carbonate. Rods were made and tested in the same way. They contained 45 parts regenerated cellulose fibers, 30 parts glue (25% solution) and 30 parts  $CaHPO_4$  powder. The filters were evaluated by test smoking as conducted in Example 4 and comparison to control filters and unfiltered cigarettes as tested in that example. The filters containing the calcium acid phosphate had an average pressure drop of 4.3 inches and their smoke contained 102 mg. tar and 16 mg. nicotine.

From the values listed above and in Example 1, it can be seen that the filter containing the combination of regenerated cellulose fibers and calcium diphosphate reduced the amount of tars collected by 37.4% and the amount of nicotine collected by 36.0%. The control filter of regenerated cellulose fibers reduced the amount of tars collected by 14.1% and the amount of nicotine collected by 16.0%. The increase in the pressure drop of the filtered cigarette due to the addition of the calcium acid phosphate to the filter was only about 5%.

In carrying out the operation of this invention, the purity of the carbonate or phosphate employed is not a critical factor. Rather, the form of its particles is more important. The salt should be in a finely powdered form so that it can be readily slurried in a liquid or passed through a spraying nozzle. While the exact size of the particle does not appear to be critical, it is indicated that the salt additive should be at least capable of passing 60 through a 200 mesh screen. Commercial grades of the salts of the invention generally may be obtained in a particle size which will pass through a 325 mesh screen. Advantageously, a salt is used which has at least 80% of its particles of a diameter less than the diameter of the fibers of the filter. For fibers of the size used in the example above, no substantial number of particles should be as large as twice the filament diameter or as small as one-tenth the filament diameter although these limits may vary considerably with fibers of other sizes. Any source of salt which passes this requirement can be employed.

While unusually good results have been obtained with filters prepared from a crimped continuous filament tow of cellulose acetate or regenerated cellulose fibers, it will be recognized by those skilled in the art that the usefulness of the invention extends to other fibrous filters, in-

cluding those prepared from fibers of cotton, nylon, polyamides, polyesters, etc., particularly where the fibers are in substantial longitudinal alignment and are coextensive with the body of the filter. It is preferred to use for filter preparation in accordance with the present invention a continuous strand, e.g. tow, of 4,000 to 35,000 filaments, the filaments being of 16 to 3 denier and having about 4 to 10 crimps per inch.

By the expression "surface solvation" as used herein is meant the creation, by the action of a solvent or plasticizer and/or heat, of an adhesive, tacky or readily bonding condition of the filaments by solution or incipient solution of surface portions of the filament material whereby there is produced a welding and adhesion between adjacent filaments contacting at such portions, and by "coalescence" is meant the situation caused by partial or incipient solvation of surface portions of the filaments and resulting in a condition within those portions under which the portions will flow into or unite with similar portions of dissolved or plastic material in contiguous filaments. Surface solvation bonds between fibers are sometimes also referred to as "fused" or "welded" bonds.

It is to be noted that while the filters of the present invention seem to derive special benefits from the chemical properties and behavior of the water-insoluble inorganic salt additives, yet the invention appears to be equally dependent upon the structural character of the filter. In this regard, the more important structural factors found in the most advantageous form of the invention seem to be:

(1) That the aligned filaments be randomly bonded at randomly spaced intervals. This may be achieved by spraying a solvent type of plasticizer onto a spread tow of synthetic thermoplastic filaments as described above. It also may be accomplished by use of a filament strand in which at least some of the filaments contain sufficient plasticizer to be softened at slightly elevated temperatures. This plasticizer may be added by spraying it onto the formed fibers or it may be added to the spinning solution before the fibers are spun.

(2) That where the additive is to be applied before or with a fiber bonding agent. In other words, no material should be employed for adhering the filaments which would coat, destroy or otherwise substantially interfere with the activity or integrity of the salt particles. That is to say, in such a case the filament bonds should be formed by coalescence of the surface solvation type. Obviously no plasticizer should be employed which has a detrimental action on the salt particles.

(3) That substantially all the salt particles be carried on the surfaces of the filaments, supported by the filaments, and substantially immobile with respect thereto. This structure is best accomplished by softening of portions of the filament surfaces with a solvent or by creating a superficial surface with a film-forming material whereby the particles may be slightly embedded in the surface or superficial surface without being coated or covered. It is also most easily accomplished when the diameters of the particles are not too different from the diameters of the filaments, the major portion of the particles being, for instance, less than twice the filament diameter, but more than one-tenth of the filament diameter.

I claim:

1. A tobacco smoke filter element comprising a bundle of continuous crimped cellulosic filaments which are generally oriented lengthwise of the filter element and extend from end to end of the filter element, a content of plasticizer for the filaments on said filaments whereby the continuous crimped filaments are bonded to one another at random points of contact, and a content of a water-insoluble salt powder from the group consisting of calcium and magnesium salts carried on and by the continuous filaments, said plasticizer also serving to bond said powdered salt to the filaments.

2. A tobacco smoke filter element comprising a bundle of continuous crimped cellulose acetate filaments, a content comprising droplets of plasticizer for the filaments on said filaments whereby the continuous cellulose acetate filaments are bonded to one another at random points of contact and a content of a powdered salt from the group consisting of calcium and magnesium salts carried on and by the continuous cellulose acetate filaments, the aforesaid plasticizer serving to bond said powdered salts to the filaments, the powdered salts being characterized in that at least 80% of the particles thereof have a diameter less than the diameter of the continuous cellulose acetate filaments and no substantial number of the powdered salt particles being as large as twice the filament diameter or as small as one-tenth the filament diameter.

3. A filter element in accordance with claim 2 wherein the cellulose acetate has a 39.2% acetyl.

4. A tobacco smoke filter element comprising a bundle of continuous crimped cellulose acetate filaments which are generally oriented lengthwise of the filter element and extend from end to end of the filter element, a content of plasticizer from the group consisting of phthalates, citrates, and propionates carried on said filaments whereby the continuous cellulose acetate filaments are bonded to one another at random points of contact and a content of salt from the group consisting of phosphates and carbonates of calcium and magnesium carried on and by the filaments, said salts being in the form of a powder smaller than 200 mesh and said plasticizer serving to bond said salt powder to the filaments.

5. A tobacco smoke filter element comprising a bundle of continuous crimped synthetic filaments, more than 10% of a bonding material compatible with the filaments carried on the filaments as droplets whereby the filaments are bonded at random points without coating of the filaments, more than 10% of a salt in powdered form from the group consisting of water-insoluble calcium and magnesium salts carried on and by said filaments, said bonding material also bonding the salt powder to the filaments whereby an improved filter element is obtained.

6. A tobacco smoke filter element comprised of more than 5000 continuous crimped cellulose acetate filaments of not more than 8 denier per filament, which filaments are generally oriented lengthwise of the filter element and extend from end to end of the filter element at least 10% plasticizer from the group consisting of phthalates, citrates, and propionates carried by said filaments, at least 20% of a powdered salt from the group consisting of water-insoluble calcium and magnesium salts carried on and by said continuous filaments, said salt powder being characterized in that at least 80% of the particles thereof have a diameter less than the diameter of the continuous cellulose acetate filaments and no substantial number of the powdered salt particles being as large as twice the filament diameter or as small as one-tenth the filament diameter.

7. A filter element in accordance with claim 1 wherein the powdered salt is from the group consisting of calcium carbonate, magnesium carbonate, calcium phosphate, magnesium phosphate, calcium pyrophosphate, magnesium pyrophosphate, calcium metaphosphate and magnesium metaphosphate.

8. A filter element consisting of a bundle of cellulose acetate continuous crimped filaments having at least about 8 crimps per inch, said filaments carrying droplets of a plasticizer from the group consisting of phthalates, citrates, and propionates, said plasticizer being present on the filaments in an amount greater than 10% by weight whereby the filaments are bonded to each other at random points of contact and the plasticized filaments carry on their surface at least 20% by weight of a powdered water insoluble salt from the group consisting of calcium and magnesium salts.

9. A tobacco smoke filter element comprising a bundle of continuous crimped synthetic filaments, more than 10% of a plasticizer as a bonding medium carried on the filaments in dispersed form whereby the filaments are bonded at random points, more than 10% of a salt in finely divided form from the group consisting of water insoluble calcium and magnesium salts carried on and by said filaments, said plasticizer also assisting in the bonding of the aforementioned finely divided salts to the filaments whereby an improved filter element is obtained. 5

10. A tobacco smoke filter element comprising a bundle of continuous crimped cellulose acetate filaments which are generally oriented lengthwise of the filter element and extend from end to end of the filter element, a content of plasticizer for cellulose acetate contained in the filaments whereby the continuous cellulose acetate filaments are bonded to one another at random points of contact, and a content of a finely divided salt from the group consisting of phosphates and carbonates of calcium 15

and magnesium carried on and by the filaments whereby an improved filter element is obtained.

References Cited in the file of this patent

UNITED STATES PATENTS

|           |                |                |
|-----------|----------------|----------------|
| 656,649   | Landfried      | Aug. 28, 1900  |
| 1,127,771 | Jones          | Feb. 9, 1915   |
| 1,784,566 | Andrews        | Dec. 9, 1930   |
| 1,936,999 | Teague         | Nov. 28, 1933  |
| 1,950,542 | Copell         | Mar. 13, 1934  |
| 2,181,614 | Striefling     | Nov. 28, 1939  |
| 2,301,159 | Drechsel       | Nov. 3, 1942   |
| 2,789,563 | Taylor et al.  | Apr. 23, 1957  |
| 2,780,228 | Touey          | Feb. 5, 1957   |
| 2,805,671 | Hackney et al. | Sept. 10, 1957 |
| 2,832,351 | Hale           | Apr. 29, 1958  |

FOREIGN PATENTS

|         |        |               |
|---------|--------|---------------|
| 813,324 | France | Feb. 22, 1937 |
|---------|--------|---------------|